# EUROPEAN PATENT SPECIFICATION

(11) **EP 0 267 681 B1**
(45) Date of publication and mention of the grant of the patent: **10.03.1993**
(21) Application number: 87308464.4
(22) Date of filing: 24.09.1987
(51) Int. Cl.: D06M 15/41

(54) **Treating fibrous polyamide articles**
Behandeln von faserigen Polyamid-Textilgebilden
Traiter des articles en polyamides fibreux

(30) Priority: 14.10.1986 US 918376
(43) Date of publication of application: 18.05.1988
(73) Proprietor: MINNESOTA MINING AND MANUFACTURING COMPANY, St. Paul, Minnesota 55133-3427 (US)
(72) Inventor: Payet, George L. c/o Minnesota Mining and, St. Paul Minnesota 55144-1000 (US); Chang, John Cheng-Chung c/o Minnesota Mining and, St. Paul Minnesota 55144-1000 (US)
(74) Representative: Wilhelm, Stefan

(56) References cited:
- EP-A- 0 026 314
- EP-A- 0 073 606
- US-A- 4 592 940
- CHEMICAL ABSTRACTS, vol. 89, 1978, page 143, abstract no. 112219x, Columbus, Ohio, US

## Description

The present invention relates to a process for providing stain resistance to polyamide articles, such as nylon and wool carpets, nylon, wool, and silk fabrics, and natural and synthetic leathers.

Fibrous polyamide articles such as nylon and wool carpets, nylon, wool, and silk fabric, natural leather, and synthetic leathers such as Ultrasuede™ are particularly susceptible to staining by natural and artificial acid colorants such as are commonly found in many foods and beverages. A need has long been felt for processes for economically providing such fibrous polyamide articles with resistance to staining by acid colorants. Particularly desirable are processes by which stain resistance can be imparted to fibrous polyamide articles during conventional processing and treating operations.

U-S-A-4,501,591 (Ucci et al.) discloses a process for providing stain-resistant polyamide carpets in which a sulfonated phenol-formaldehyde condensation product and an alkali metal silicate are added to the dye liquor in a continuous dyeing process, followed by steaming, washing, and drying the carpet.

US-A-4,592,940 (Blyth et al.) discloses a process for imparting stain resistance to nylon carpet by immersing the carpet in a boiling aqueous solution of a selected phenol-formaldehyde condensation product at a pH of 4.5 or less. The process is carried out in conventional beck dyeing apparatus subsequent to dyeing (generally at a pH of 6.5 to 8.0) by either acidifying the bath to pH 4.5 or less or draining the dye bath and then replacing the dye bath with a corresponding amount of water adjusted to pH 4.5 or less. Blyth et al. disclose that insufficient condensation product for imparting stain resistance is picked up by the carpet at pH greater than 4.5 and temperature less than 95°C.

US-A-4,579,762 (Ucci) discloses stain-resistant nylon carpet in which the nylon fibers are made from polymer modified to contain, as an integral part of its polymer chain, sufficient aromatic sulfonate units to improve the acid dye resistance of the fibers and in which the backing adhesive contains a fluorochemical in an amount sufficient to render the backing a barrier to liquids.

Japanese Examined Patent Application (Kokoku) No. 48-8789 (1973) (Meisei) discloses a method for treatment of dyed polyamide fibers to improve anti-static and anti-melting properties and moisture resistance in which a ligand oligomer, formed from sulfonated 4,4ʹ-dihydroxy-diphenyl sulfone-formaldehyde condensate with a metal compound prepared from citric acid and a metal chloride, metal oxide, or organic metal salt, is applied to fiber from a treatment bath or, alternatively, the sulfonated 4,4ʹ-dihydroxy-diphenyl sulfone-formaldehyde condensate and a metal compound prepared from a metal salt, citric acid and hydroxy acetic acid, are added to the treatment bath separately.

US-A-4,329,391 (McAlister) discloses the treatment of synthetic fibers with a sulfonated polyester stain-releasing finish in an aqueous bath which includes the addition of water-soluble salts to the aqueous fabric treating bath. The treatment provides a finish which enhances oily soil release during after-stain laundering.

U.S. Defensive Publication T949,001 (Pacifici) discloses a process for improving the durability of water-dispersible polyester and polyester amide textile finishes on fabric where the fabric, after application of the finish, is treated with an aqueous solution of polyvalent metal salts.

US-A-3,322,488 (Feeman) discloses sulfomethylated condensation products of bisphenols and aldehydes for use in reserving synthetic polyamide and polyurethane fibers to render them resistant to acid and direct dyes.

US-A-3,663,157 (Gilgien et al.) discloses a process for printing nylon fabric with disperse or monosulfonated acid dyes wherein the fabric is pretreated with an aqueous solution of a fiber-substantive, water-soluble, anionic resist which is a polycondensate of a diarylsulfone containing at least one phenolic hydroxy group with formaldehyde.

US-A-3,926,548 (Moriyama et al.) discloses aminated hydrophobic fibers having a surface resistant to anionic dyes, the surface of the fibers having been treated with a compound having groups capable of linking to amino groups in the fibers to form covalent bonds. Such groups include halotriazinyl, halopyrimidinyl, haloquinoxalyl, haloacrylamido, vinylsulfo groups, etc., or any other groups that can produce these groups. Also suitable are compounds having anionic groups, for example, sulfonate, carboxylate, sulfate, phosphate groups, etc., besides the highly reactive groups capable of reacting with amino groups.

US-A-3,959,559 (Kimoto et al.) discloses a process for producing modified synthetic fibers in which the fibers are treated with a reaction product of a specified s-triazine or piperazine derivative, with a specified derivative of polyoxyethylene and further adhering onto the resulting fibers a specified aromatic sulfonic acid. The modified fibers resist contamination from liberated dyestuff or ionic contaminants during laundering or dry cleaning.

US-A-4,322,512 (Lenox) discloses treating a polyamide textile material with a substituted trimellitic anhydride compound, the treatment decreasing the textile material's affinity for acid dyes.

US-A-4,343,923 (Lenox et al.) discloses a method for decreasing a textile material's affinity for acid dyes in which the textile material is pretreated with an acylimidazole compound.

Brownewell, Ralph G., "Two New Chemicals Create Better Multicolored Nylons," American Dyestuff Reporter, Vol. 68, No. 3, 1979, pp 38-41, discloses processes for providing nylon fabrics which are resistant to coloration by acid dyes by treatment with Sandospace S, a product of Sandoz Colors and Chemicals, believed to be a benzenoid triazine derivative.

US-A-4,563,190 (Topfl) discloses a dyeing assistant useful in the dyeing of polyamide fibers with acid dyes. The dyeing assistant is a mixture of (A) a sulfonated condensation product of hydroxyaryl compounds and formaldehyde or a sulfonated N-aryl-melamine derivative, and (B) a specified quaternary ammonium, and, optionally, (C) a siloxane/oxyalkylene copolymer and (D) a polar solvent.

EP-A-0 102 690 discloses increased exhaustion of fluorochemical treating agents for providing oil and water repellency by the addition of salt compounds such as sodium sulfate and citrate, magnesium chloride, ammonium sulfate and chloride, aluminum sulfate, calcium chloride, and potassium chloride.

US-A-4,013,627 (Temple) discloses a fluorochemical polymer for treating fabrics to provide oil and water repellency, the polymer being derived from fluorochemical acrylate monomer, a vinyl monomer free of non-vinylic fluorine, and a vinyl monomer which contains an onium ionic group. Salts, such as alkali metal sulfates and low molecular weight alkylamine hydrochlorides, may be added, as adjuvants, to textile treating baths containing the fluorochemical polymer to aid deposition of the polymer onto the fabric being treated.

EP-A-0,016,658 (Monsanto) discloses soil-resistant carpet yarns prepared by coating the yarn with a soil retardant agent such as a fluorochemical and a retaining agent such as zirconium oxide.

U.S. Patent No. 4,592,940 (Blyth et al.) discloses nylon carpets which are rendered resistant to staining normally caused by artificial colorants such as F,D&C Red Dye No. 40 by immersing the carpets ion a boiling aqueous solution of a selected phenol-formaldehyde condensation product at a pH of 4.5 or less. A particularly useful condensation product reported is that obtained by the condensation of formaldehyde with a mixture of diphenolsulfone and phenolsulfonic acid.

Japanese Kokai No. 52[1977]-155300 (Kuraray) discloses a composition for flameproofing synthetic fabrics, such as nylon and polyester, having as a major component prepared by bonding a compound represented by the general formula
(wherein X is COOH or SO₃H or salts thereof and Y is COOH SO3H, H or a group which is inactive to methlolconversion reaction) and formaldehyde which component has a methylol conversion degree of 1 to 3 and a degree of number average polymerization of 1 to 2.

The present invention provides a method for providing fibrous polyamide material with stain resistance to natural and artificial acid colorants comprising contacting the fibrous polyamide material with an aqueous solution comprising a normally solid, water-soluble, partially sulfonated novolak resin, which comprises the condensation product of at least one phenolic compound and an aldehyde such as, for example, formaldehyde or acetaldehyde, and a water-soluble divalent metal salt. The resin and salt other than that of a phenol/aldehyde condensation product are applied in sufficient amounts and for sufficient time at a given temperature to provide stain resistance. The combination of the sulfonated novolak resin and divalent metal salt provides surprising effective stain resistance using reduced amounts of the resin and permits application over a wide pH range.

The method of this invention can be carried out in three different ways. One method comprises the steps of
Ia) adding to a dyebath, before, during, or after dyeing of the fibrous polyamide material, such as in a dye beck with nylon carpet, at least 0.1% solids based on the weight of the fabric (owf) of the sulfonated novolak resin and at least 1% owf of the divalent metal salt,
Ib) immersing the polyamide material in the dyebath for a time and temperature sufficient to exhaust the sulfonated novolak resin onto the polyamide material,
Ic) removing the treated polyamide material from the dyebath, and
Id) drying the removed polyamide material.

A second method comprises the steps of
IIa) applying to the polyamide material an aqueous solution comprising at least 0.1% solids owf of the sulfonated novolak resin and at least 1% owf of the divalent metal salt, such as during continuous dyeing of nylon carpet using Kuster™ or Otting™ continuous dyeing equipment,
IIb) steaming the treated polyamide material for a time sufficient to effect adherence of the sulfonated novolak resin to the polyamide material, and
IIc) drying the polyamide material.

A third method comprises the steps of
IIIa) padding an aqueous solution comprising at least 0.1% owf of the sulfonated novolak resin and at least 1% owf of the divalent metal salt onto the polyamide material and
IIIb) drying the polyamide material.

The invention further provides including a fluorochemical composition in the aqueous solution comprising the sulfonated novolak resin and the divalent salt in step Ia, IIa, or IIIa to provide the polyamide material with oil and water repellency. The invention further provides an aqueous solution useful in providing stain resistance to fibrous polyamide material comprising the water-soluble partially sulfonated novolak resin and the water-soluble divalent salt. The invention also provides fibrous polyamide materials such as nylon, silk, and wool fabrics, yarns, and fibers, nylon and wool carpets, and natural and synthetic leather such as Ultrasuede™ with stain resistance by treating the polyamide materials as described in method I, II, or III hereinabove.

The present invention still further provides fibrous polyamide materials with stain resistance and oil and water repellency by treating the polyamide material, as described in method I, II, or III hereinabove, with a fluorochemical composition added to the treating solution.

The sulfonated novolak resins useful in this invention include known substances such as those compositions which are condensation products of formaldehyde with bis(hydroxyphenyl)sulfone and phenylsulfonic acid. Instead of, or in addition to, formaldehyde, another aldehyde such as, for example, acetaldehyde, furfuraldehyde, or benzaldehyde, can be used to make the condensation product. Also, other phenolic compounds such as, for example, bis(hydroxyphenyl)alkane, e.g., 2,2-bis(hydroxyphenyl)propane, and bis(hydroxyphenyl) ether compounds can be used instead of, or in addition to the bis(hydroxyphenyl)sulfone. The sulfonated novolak resin is partially sulfonated, i.e., has a sulfonic acid equivalent weight of about 300-1200, preferably 400-900. Examples of such resins are disclosed in U.S. Patent No. 4,592,940 (Blyth et al.) which is incorporated herein by reference for this purpose. Also commercially available sulfonated novolak products are available such as Intratex™ N, available from Crompton and Knowles Corp., and Erional™ PA, available from Ciba-Geigy Corp., Nylofixan™P available from Sandoz Ltd. Mesitol™ NBS, available from Mobay Chemical Corp., Resist #4, available from Lyndal Chemical Co., Ameriolate™, available from American Emulsions Co. Inc. and Synthabond™ 1938 available from Piedmont Chemical Industries. Sulfonation of phenolic compounds is taught, for example, in Sulfonated and Related Reactions, E. E. Gilbert, Interscience Publishers, (1965). Condensation of phenol-formaldehyde resins is taught, for example, in Phenolic Resins, A. Knop et al., Springer-Verlag, (1985).

The divalent metal salts useful in the present invention include water soluble inorganic and organic salts of metals such as magnesium, barium, calcium, and zinc. Inorganic metal salts include chlorides, sulfates, and nitrates of these metals. Organic metal salts include acetates and formates of these metals. Preferred divalent metal salts are magnesium sulfate, magnesium chloride and magnesium acetate. Mixtures of two or more salts can also be used in this invention. Generally, when both the sulfonated novolak resin and fluorochemical compositions are in the aqueous treating solution, magnesium salts are preferably used to achieve both stain resistance and oil and water repellency.

The fluorochemical compositions useful in the present invention for providing oil and water repellency include anionic, cationic, or nonionic fluorochemicals such as the fluorochemical allophanates disclosed in U.S. Patent No. 4,606,737 (Stern); fluorochemical polyacrylates disclosed in U.S. Patent Nos. 3,574,791 (Sherman et al.) and 4,147,851 (Raynolds); fluorochemical urethanes disclosed in U.S. Patent No. 3,398,182 (Guenthner et al.); fluorochemical carbodiimides disclosed in U.S. Patent No. 4,024,178 (Landucci); fluorochemical guanidines disclosed in U.S. Patent No. 4,540,497 (Chang et al.).

The sulfonated novolak resins are preferably used in an amount of at least 0.1% solids owf, more preferably 0.15% owf, most preferably at least 0.35% owf. Amounts in excess of 3% owf generally do not provide any appreciable increase in stain resistance. The amount of sulfonated novolak resin required to provide adequate stain resistance depends on the fibrous polyamide material being treated. For example, nylon 6 and wool generally require larger amounts of the resin than nylon 66. When the polyamide material is heat-set carpet yarn, yarn heat-set under moist conditions, e.g., in an autoclave, generally requires larger amounts of the resin than with yarn heat-set under substantially dry conditions.

The divalent metal salts are preferably used in an amount of at least 1% owf, more preferably at least 1.5% solids owf, most preferably at least 2% solids. Amounts of the salt in excess of 5% owf generally do not provide any appreciable increase in stain resistance.

The fluorochemical composition, when included in the treating solution, is preferably present in an amount of at least about 0.15% solids owf, more preferably at least 0.2% solids owf, most preferably 0.35% owf. Generally, amounts of the fluorochemical composition in excess of 2% solids owf do not appreciably improve the oil and water repellency. Generally, when the polyamide material is nylon fiber, smaller denier fiber requires larger amounts of the fluorochemical composition than larger denier fiber.

The sulfonated novolak resin and water-soluble divalent metal salt can be applied from an aqueous exhaust bath such as is used in beck dyeing of carpet. The sulfonated novolak resin and the water soluble divalent metal salt can be added to the aqueous dye bath solution and exhausted concurrently with the dye. Generally, the dye bath is maintained at a temperature at or near the boiling point for a period of 10 to 90 minutes or more to effect exhaustion of the dye and the sulfonated novolak resin. Surprisingly, the dye bath can be maintained in the normal pH rang of 4.5 to 8.0 with excellent results. Dye bath pH can range from 2.0 to 12.0, although pH in the range of 4 to 7 is preferred.

Alternatively, the sulfonated novolak resin and the water-soluble divalent metal salt can be added to the aqueous dye bath after exhaustion of the dye or the dyebath can be drained and fresh water added prior to the addition of the sulfonated novolak resin and the water-soluble divalent metal salt. Generally, the resin/salt bath is maintained at a temperature at or near boiling for a period of time sufficient to exhaust the resin, usually 10 to 90 minutes.

The sulfonated novolak resin and divalent metal salt can be applied during continuous dyeing, such as with Kuster™ or Otting™ carpet dyeing equipment. The sulfonated novolak resin and the water-soluble divalent metal salt can be added directly to the aqueous dye solution and the solution is conventionally applied to the polyamide carpet. Alternatively, the sulfonated novolak resin and the water-soluble metal salt can be applied during a wetting out step prior to application of the dye. The carpet is then steamed, as usual, for 3 to 5 minutes.

The sulfonated novolak resin and divalent salt can also be applied to polyamide material by a padding operation. This can be done as a separate step or in conjunction with the application of various convention finishes such as wetting agents, softeners, and leveling agents. After application of the resin/salt solution, the polyamide material is conventionally dried.

Fluorochemical compositions for providing oil and water repellency can also be applied in conjunction with the sulfonated novolak resin. The fluorochemical composition is simply added in an appropriate amount to the treating solution. In some cases, particularly in exhaust applications, useful divalent metal salts may be limited to the inorganic and organic magnesium salts.

The following non-limiting examples serve to illustrate the invention. In the following examples, all ratios are by weight and percentages are weight percent unless otherwise indicated. In the examples where the material being treated is nylon 66 carpet, the carpet is scoured, greige, unbacked, level-loop carpet.

### Preparation of a sulfonated phenol-formaldehyde resin (hereinafter SPFR):

To a three-neck flask, fitted with a mechanical stirrer, thermometer, and condenser, was added 473 g of acetic anhydride and 945 g of 4,4ʹ-dihydroxydiphenylsulfone (DDS). Then 473 g of conc. sulfuric acid was added via a dropping funnel over a period of one hour with stirring. The resulting reaction mixture was heated and stirred at 100°C for 7 hours. Water (340 g) was added in portions while distilling off acetic acid over one hour. After addition of 250 g of 37% aqueous formaldehyde and 338 g of water, the reaction mixture was heated to 100°C for 6 hours. The resulting sulfonated 4,4ʹ-dihydroxydiphenylsulfone-formaldehyde condensate was diluted with 1400 g of water and neutralized to a pH of 6.0 with 550 g of 5% NaOH to yield the sodium salt of the partially sulfonated novolak resin product as a 36% aqueous concentrate (SPFR).

In the following examples, fibrous polyamide materials were evaluated using the following test methods:

### Stain Resistance (SR)

A 1 g sample of the fibrous polyamide material under evaluation is placed in 40 ml aqueous solution containing 0.008 weight percent FD&C Red Dye No. 40 and 0.04 weight percent citric acid at room temperature (22°C) and agitated for one hour. The sample is removed from the dye solution, rinsed and blotted with paper towels to remove excess moisture. The amount of staining is evaluated visually using a rating scale which ranges from 1-5, where 1 is essentially unstained and 5 is heavily stained. Generally, a stain resistance of less than 3 is satisfactory.

### Water Repellency (WR)

The water repellency of treated polyamide samples is measured using a water/isopropyl alcohol test, and is expressed in terms of a water repellency rating on a scale of 0 to 10 of the treated carpet or fabric. Treated carpets which are penetrated by or resistant only to a 100 percent water/0 percent isopropyl alcohol mixture (the least penetrating of the test mixtures) are given a rating of 0, whereas treated fabrics resistant to a 0 percent water/100 percent isopropyl alcohol mixture (the most penetrating of the test mixtures) are given a rating of 10. Other intermediate values are determined by use of other water/isopropyl alcohol mixtures, in which the percentage amounts of water and isopropyl alcohol are each multiples of 10. The water repellency rating corresponds to the most penetrating mixture which does not penetrate or wet the fabric after 10 seconds contact. In general, a water repellency rating of at least 1, is desirable for carpet.

### Oil Repellency (OR)

The oil repellency of the treated polyamide samples is measured by AATCC Standard Test 188-1978, which test is based on the resistance of treated fabric to penetration by oils of varying surface tensions. Treated fabrics resistant only to Nujol™, a brand of mineral oil and the least penetrating of the test oils, are given a rating of 1, whereas treated fabrics resistant to heptane (the most penetrating of the test oils) are given a value of 8. Other intermediate values are determined by use of other pure oils or mixtures of oils. The rated oil repellency corresponds to the most penetrating oil (or mixture of oils) which does not penetrate or wet the fabric after 10 seconds contact rather than the 30 seconds contact of the Standard Test. Higher numbers indicate better oil repellency. Additionally, a value of 0 indicates no resistance to Nujol™. In general, an oil repellency of at least 1 or greater is desirable for carpet.

### Examples 1-3 and Comparative Example C1-C4

Samples of nylon 66 carpet which had been heat-set for 10 minutes at 150°C under substantially dry conditions, were immersed in an aqueous bath containing 0.3% solids SPFR and the amount of various salts shown in Table 1. A 20:1 liquor to fabric ratio, a pH of 6 a bath temperature of 97°C, and a treatment time of 90 minutes were used. The carpet samples were removed from the bath, rinsed, and dried for 10 minutes at 70°C and then for 5 minutes at 130°C. The carpet samples, together with a carpet sample to which no SPFR and no salt were added (Comparative Example C1), were tested for stain resistance (SR). The results are shown in Table 1.

As can be seen from the data in Table 1, the use of divalent magnesium salts provides significantly better stain resistance to the carpet than does the use of the monovalent salts, ammonium sulfate and sodium chloride, even when relatively large amounts (5% owf) of the monovalent salts are used.

### Examples 4-8 and Comparative Examples C5-C9

In Examples 4-7, samples of nylon 66 carpet which had been heat-set for 10 minutes at 150°C under substantially dry conditions, were immersed for 90 minutes in an aqueous solution at 97°C and a pH of 6 and a liquor to fabric ratio of 20:1 using 0.2% owf SPFR with 2% solids owf of various salts. In Comparative Example C5, no SPFR or salt were used and, in Comparative Example C6, SPFR was used without salt. In Example 8 and Comparative Examples C7-C9, 0.25% owf of a fluorochemical oil, and water repellent composition, FX-364, available from 3M Company, was added to the treating solution containing SPFR and salt. Each sample was removed from the solution, rinsed, and dried for 10 minutes at 70°C and then for 5 minutes at 130°C. Each sample was tested for stain resistance (SR), oil repellency (OR), and water repellency (WR). The results are shown in Table 2.

As can be seen from the results in Table 2, each of the samples treated with SPFR have good stain resistance when used with the indicated divalent metal salts although very little stain resistance resulted from the SPFR alone at this concentration. When the fluorochemical was added, oil and water repellency were achieved when MgCl₂, CaCl₂, and ZnCl₂ were present and adequate stain resistance was achieved only with MgCl₂ (Example 8).

### Examples 9-10 and Comparative Examples C10-C11

Samples of nylon carpet which had been heat-set for 10 minutes at 150°C under substantially dry conditions, were dyed by immersion in an aqueous bath using 0.25% owf Tectilon™ Blue 5GS, available from Ciba-Geigy Corp., without SPFR, with 0.15% solids owf SPFR only added, and with 0.15% solids owf SPFR and 2% owf MgCl₂ added. In Comparative Example C6 only water was used. on each, a liquor to fabric ratio of 20:1, a bath temperature of 97°C, a pH of 6 and a treatment time of 90 minutes were used. The dye exhausted well in each example to provide a level blue shade. Each sample was removed from the bath, rinsed, and dried for 10 minutes at 70°C and then 5 minutes at 130°C. Each sample was evaluated for stain resistance (SR). The aqueous dye bath constituents and stain resistance are shown in Table 3.

As can be seen in Table 3, only when both the SPFR and MgCl₂ were present was excellent stain resistance achieved at this concentration of SPFR.

### Examples 11 and 12 and Comparative Examples C12-C16

Samples of wool gabardine fabric were immersed in an aqueous solution of SPFR and 2.0% owf magnesium acetate as set forth in Table 4. For each sample, a liquor to fabric ratio of 20:1, treatment temperature of 97°C, a pH of about 6 and a treatment time of 90 minutes were used. Each sample was removed from the treating solution, rinsed, and dried for 10 minutes at 70°C and then for 5 minutes at 130°C. Each sample was tested for stain resistance (SR). The results are shown in Table 4.

As can be seen from the results in Table 4, good stain resistance is achieved on wool gabardine at SPFR concentration of 0.30% owf and above when magnesium acetate was present. No stain resistance was shown when the salt was not used.

### Examples 13-14 and Comparative Examples C17-C18

Samples of chamois (natural leather) and upholstery-weight, nylon Ultrasuede™ (synthetic leather) were treated by immersing the sample in water or in aqueous solutions containing 0.35% solids owf SPFR and 2% owf magnesium acetate at room temperature at a liquor to fabric ratio of 20:1 for 46 hours. Each sample was removed from the treating solution, rinsed and dried for 10 minutes at 70°C and then for 5 minutes at 130°C. Each sample was tested for stain resistance (SR), the results are set forth in Table 5.

As can be seen from the data in Table 5, excellent stain resistance can be achieved with both natural and synthetic leather when both SPFR and salt are present in the treatment bath.

### Examples 15-24 and Comparative Examples C18-C29

Samples of nylon 66 level loop carpet which had been heat-set for 10 minutes at 150°C under substantially dry conditions, were dyed by immersing the samples in aqueous solutions at various pH's using 0.35% solids owf SPFR with and without 2% owf magnesium acetate at a liquor to fabric ratio of 20:1, a treatment temperature of 97°C, a pH of about 6 and a treatment time of 90 minutes in a Launderometer. A sample also was treated with water only. Each sample was removed from the treating solution, rinsed, and dried for 10 minutes at 70°C and then for 5 minutes at 130°C. Each sample was tested for stain resistance (SR). The results are shown in Table 6.

The data in Table 6 show that the good stain resistance obtained with SPFR at pH values of 3-6 is improved by the addition of magnesium acetate. At pH values of 7-10, the poor stain resistance seen with the use of only SPFR is improved to acceptable stain resistance ratings with the addition of magnesium acetate.

### Examples 25-27 and Comparative Examples C30-C32

In these Examples, nylon upholstery fabric which had been heat-set for 10 minutes at 150° under substantially dry conditions, was treated by padding (50% wet pick up) an aqueous solution containing 0.3% solids owf SPFR with and without 2% owf magnesium chloride salt, and with and without a 0.3% solids owf of a blend of fluorochemical oil and water repellent composition, FC-214, available from 3M Company (FC). Each sample was dried for 10 minutes at 70°C and then for 5 minutes at 130°C. Each sample was tested for stain resistance (SR), oil repellency (OR), and water repellency (WR). The results are shown in Table 7.

As can be seen from the data in Table 7, when the magnesium chloride salt was present with the SPFR and the fluorochemical composition, acceptable oil and water repellency (rating of at least 1) and improved stain resistance (rating of 1-1.5) where achieved.

### Examples 28-42 and Comparative Examples C33-C48

In these examples, samples of nylon 66 level loop carpet which had been heat-set under substantially dry conditions for 1 minute at 200°C, were treated by immersion in an aqueous bath at a liquor to fabric ratio of 21.5:1, at treating temperature of 97°C, and a treatment time of 90 minutes with 0.3% solids owf SPFR various commercial novolak resins (NR) with and without 2% owf magnesium chloride and with and without 0.25% solids owf of a fluorochemical composition, FX-364, available from 3M Company (FC). The pH was adjusted to 3.5 with acetic acid. The samples were removed from the treating solution, rinsed, and dried for 10 minutes at 70°C and then for 5 minutes at 130°C. The samples were tested for stain resistane (SR), oil repellency (OR), and water repellency (WR). The results are shown in Table 8.

### Examples 43-48 and Comparative Examples C49-C51

Samples of nylon 66 level loop carpet which had been heat-set under substantially dry conditions for 10 minutes at 150°C, were treated by immersion in an aqueous solution containing 0.5% solids owf SPFR, with and without 20% owf magnesium sulfate salt, with and without 0.5% solids owf fluorochemical oil and water repellent (FC), and with and without Tectilon™ Blue 5GS dye, available from Ciba-Geigy Corp., as indicated in Table 9. Treatment was carried out at a pH of 4.5, a liquor to fabric ratio of 20:1, a treatment temperature of 97°C, and a treatment time of 90 minutes. Comparative Example C49 was prepared using no SPFR, salt, fluorochemical, or dye. Each sample was removed from the treating solution, rinsed and dried at 70°C for 10 minutes then at 130°C for 5 minutes. Each sample was tested for stain resistance (SR), oil repellency (OR) and water repellency (WR). The results are shown in Table 9.

As can be seen from Table 9, excellent stain resistance and oil and water repellency are achieved only when the salt is present as in Examples 43-48. Each dyed sample was levelly dyed to the expected depth based on the amount of dye present.

### Example 49 and Comparative Examples C52-C53

Samples of nylon 66 level loop carpet which had been heat-set under substantially dry conditions for 1 minute at 200°C, were laboratory dyed using a procedure which simulates continuous carpet dyeing. Dye formulations containing 0.5 g/l Karawet™ DOSS, available from Lyndal Chemical Co., 0.25 g/l Sequesterent™ 220, available from Ciba-Geigy Corp., 0.1 g/l sodium thiosulfate, 0.026 g/l Tectilon™ Blue 4R200, 0.032 g/l Tectilon™ Red 2B200, and 0.050 g/l Tectilon™ Orange 3G200, each dye available from Ciba-Geigy Corp., with and without 0.35% solids owf SPFR and with and without 2% owf magnesium chloride were applied to the samples by pressing the samples face down in a tray containing the dye solution after the samples were wet-out with a 2 g/l aqueous solution of Karawet™ DOSS. The dye bath pH was 6.0. The carpet was removed from the dye bath and steamed at 100°C, 100% r.h. for 5 minutes, dried for 20 minutes at 70°C. and set at 130°C for 10 minutes. The samples were tested for stain resistance. The results are shown in Table 10.

The results in Table 10 show that only when the salt is present, is excellent stain resistance achieved.

Various modifications and alterations of this invention will be apparent to those skilled in the art without departing from the scope of this invention and this invention should not be restricted to that set forth herein for illustrative purposes.

## Claims

1. A method for providing fibrous polyamide materials with stain resistance comprising contacting the fibrous polyamide materials with an aqueous solution comprising a normally solid, water-soluble, partially sulfonated novolak resin, which comprises the condensation product of at least one phenolic compound and an aldehyde characterized in that said solution further contains a water-soluble salt of a divalent metal other than that of a phenol/aldehyde condensation product.

2. The method of claim 1 comprising adding to a dyebath, before, during or after dyeing of the polyamide material, at least 0.1% solids based on the weight of the polyamide material of said sulfonated novolak resin and at least 1% based on the weight of the polyamide material of said water-soluble salt of a divalent metal, immersing the polyamide material in the dyebath for a time and temperature sufficient to exhaust the sulfonated novolak resin onto the polyamide material, removing the polyamide material from the dyebath and drying the polyamide material.

3. The method of claim 1 comprising applying to the polyamide material a solution comprising at least 0.1% solids based on the weight of the polyamide material of said sulfonated novolak resin and at least 1% of said water-soluble salt of a divalent metal based on the weight of the polyamide material, steaming said polyamide material for a time sufficient to effect adherence of said sulfonated novolak resin to said polyamide material, and drying the polyamide material.

4. The method of claim 1 comprising padding a solution comprising at least 0.1% based on the weight of the polyamide material of said sulfonated novolak resin and 1% based on the weight of the polyamide material of said water-soluble salt of a divalent metal onto the polyamide material and drying the polyamide material.

5. The method of claim 1 wherein said water-soluble salt of a divalent metal is selected from inorganic and organic salts of magnesium, barium, calcium, and zinc.

6. The method of claim 1 wherein said sulfonated novolak resin comprises a sulfonated condensation product of at least one phenolic compound and an aldehyde.

7. The method of claim 1 wherein said aqueous solution further contains a fluorochemical oil and water repellent composition and said water-soluble metal salt is a magnesium salt.

8. A fibrous polyamide material treated according to the method of claim 1.

9. An aqueous solution for providing stain resistance to fibrous polyamide materials, said solution comprising a normally solid, water-soluble, partially sulfonated novolak resin characterized in that said solution further contains a water-soluble salt of a divalent metal other than that of a phenol/aldehyde condensation product.

10. The solution of claim 9 wherein said solution comprises at least 0.1% solids based on the weight of the polyamide material of said sulfonated novolak resin and at least 1% of said water-soluble salt of a divalent metal based on the weight of the polyamide material.

11. The solution of claim 9 wherein said solution further comprises a fluorochemical oil and water repellent composition.

## Patentansprüche

1. Verfahren zum Herstellen von verfärbungsbeständigen Polyamid-Fasermaterialien, in dem die Polyamid Fasermaterialien mit einer wäßrigen Lösung kontaktiert werden, die ein normalerweise festes, wasserlösliches, teilsulfoniertes Novolakharz enthält, das wenigstens teilweise aus dem Kondensationsprodukt mindestens einer Phanolverbindung und eines Aldehyds besteht, dadurch gekennzeichnet, daß die Lösung ferner ein wasserlösliches Salz eines zweiwertigen Metallsalzes enthalt, das kein Salz eines Phenol-Aldehyd-Kondensationsprodukts ist.

2. Verfahren nach Anspruch 1, in dem zu einem Färbebad vor oder nach dem Färben des Polyamidmaterials oder während dieses Färbens eststoff des sulfonierten Novolakharzes in einer Menge von mindestens 0,1 Gew.-%, des Polyamidmaterials und das wasserlösliche Salz eines zweiwertigen Metalls in einer Menge von mindestens 1 Gew.-% des Polyamidmatarials zugesetzt werden, das Polyamidmaterial in das Färbebad solange und bei einer solchen Temperatur getaucht wird, daß das sulfonierte Novolakharz auf dem Polyamidmatarial abgeschieden wird, das Polyamidmaterial dem Färbebad entnommen und das Polyamidmaterial getrocknet wird.

3. Verfahren nach Anspruch 1, in dem auf das Polyamidmaterial eine Lösung aufgetragen wird, die Festatoff des sulfonierten Novolakharzes in einer Menge von mindestens 0,1 Gew.-% das Polyamidmaterials und das wasserlösliche Salz eines zweiwertigen Metalls in einer Menge von mindestens 1 Gew.-% des Polyamidmaterials enthält, das Polyamidmaterial solange gedämoft wird, daß das sulfonierte Novolakharz an dem Polyamidmaterial haftet, und das Polyamidmaterial getrocknet wird.

4. Verfahren nach Anspruch 1, dadurch gekennzeichnet, daß auf das Polyamidmaterial eine Lösung aufgeklotzt wird, die Feststoff des sulfonierten Novolakharzes in einer Menge von mindestens 0,1 Gew.-% des Polyamidmaterials und das wasserlösliche Salz eines zweiwertigen Metalls in einer Menge von mindestens 1 Gew.-% des Polyamidmaterials enthält.

5. Verfahren nach Anspruch 1, dadurch gekennzeichnet, daß das wasserlösliche Salz eines zweiwertigen Metalls aus den anorganischen und organischen Salzen des Magnesiums, Bariums, Calciums und Zinks ausgewählt wird.

6. Verfahren nach Anspruch 1, dadurch gekennzeichnet, daß das sulfonierte Novolakharz wenigstens teilweise aus einem sulfonierten Kondensationsprodukt mindestens einer Phenolverbindung und eines Aldehyds besteht.

7. Verfahren nach Anspruch 1, dadurch gekennzeichnet, den die wäßrige Lösung ferner eine öl- und wasserabweisende fluorchemische Zusammensetzung enthält und daß das wasserlösliche Metallsalz ein Magnesiumsalz ist.

8. Polyamidfasermaterial, das nach dem Verfahren nach Anspruch 1 behandelt worden ist.

9. Wäßrige Lösung vom Verfärbungsbeständigmachen von Polyamidfasermaterialien, die ein normalerweise festes, wasserlösliches, teilsulfoniertes Novolakharz enthält, dadurch gekennzeichnet, daß die Lösung ferner ein wasserlösliches Salz eines zweiwertigen Metalls enthält, das kein Salz eines Phenol-Aldehyd-Kondensationsprodukts ist.

10. Lösung anch Anspruch 9, dadurch gekennzeichnet, daß die Lösung Feststoff des sulfonierten Novolakharzes in einer Menge von mindestens 0,1 Gew.-% des Polyamid-materials und das wasserlösliche Salz eines zweiwertigen Metalls in einer Menge von mindestens 1 Gew.-% des Polyamidmaterials enthält.

11. Lösung anch Anspruch 9, dadurch gekennzeichnet, daß die Lösung ferner eine öl- und wasserabweisende fluorchemische Zusammensetzung enthält.

## Revendications

1. Procédé pour donner à des matières en polyamides fibreux une résistance aux saletés, comprenant la mise en contact des matières en polyamides fibreux avec une solution aqueuse comprenant une résine novolaque partiellement sulfonée, soluble dans l'eau, normalement solide, qui comprend le produit de condensation d'au moins un composé phénolique et d'un aldéhyde, caractérisé en ce que cette solution contient en outre un sel soluble dans l'eau d'un métal divalent autre que celui d'un produit de condensation de phénol/aldéhyde.

2. Procédé suivant la revendication 1, comprenant l'addition à un bain de teinture, avant, durant ou après la teinture de la matière en polyamide, d'au moins 0,1 % de matières solides, par rapport au poids de la matière en polyamide, de la résine novolaque sulfonée susdite, et d'au moins 1 %_{,} par rapport au poids de la matière en polyamide, du sel susdit, soluble dans l'eau, d'un métal divalent, l'immersion de la matière en polyamide dans le bain de teinture pendant une période de temps et à une température suffisantes pour épuiser la résine novolaque sulfonée sur la matière en polyamide, l'enlèvement de la matière en polyamide hors du bain de teinture, et le séchage de cette matière en polyamide.

3. Procédé suivant la revendication 1, comprenant l'application, à la matière en polyamide, d'une solution comprenant au moins 0,1 % de matières solides, par rapport au poids de la matière en polyamide, de la résine novolaque sulfonée précitée, et au moins 1 % du sel soluble dans l'eau susdit d'un métal divalent, par rapport au poids de la matière en polyamide, le traitement à la vapeur d'eau de la matière en polyamide susdite pendant une période de temps suffisante pour provoquer l'adhérence de cette résine novolaque sulfonée à la matière en polyamide, et le séchage de cette dernière.

4. Procédé suivant la revendication 1, comprenant l'imprégnation d'une solution comprenant au moins 0,1 %_{,} par rapport au poids de la matière en polyamide, de la résine novolaque sulfonée précitée, et au moins 1 %_{,} par rapport au poids de la matière en polyamide, du sel soluble dans l'eau susdit d'un métal divalent, sur la matière en polyamide, et le séchage de cette dernière.

5. Procédé suivant la revendication 1, dans lequel le sel soluble dans l'eau précité d'un métal divalent est choisi parmi les sels inorganiques et organiques de magnésium, de baryum, de calcium et de zinc.

6. Procédé suivant la revendication 1, dans lequel la résine de novolaque sulfonée consiste en un produit de condensation sulfoné d'au moins un composé phénolique et d'un aldéhyde.

7. Procédé suivant la revendication 1, dans lequel la solution aqueuse précitée contient en outre une composition fluorochimique repoussant l'huile et l'eau, et le sel de métal soluble dans l'eau susdit est un sel de magnésium.

8. Matière en polyamide fibreux, traitée suivant le procédé de la revendication 1.

9. Solution aqueuse pour donner une résistance aux taches à des matières en polyamides fibreux, cette solution comprenant une résine novolaque, partiellement sulfonée, soluble dans l'eau, normalement solide, cette solution étant caractérisée en ce qu'elle contient en outre un sel soluble dans l'eau d'un métal divalent, autre que celui d'un produit de condensation de phénol/ aldéhyde.

10. Solution suivant la revendication 9, qui comprend au moins 0,1 % de matières solides, par rapport au poids de la matière en polyamide, de la résine novolaque sulfonée précitée et au moins 1 % du sel soluble susdit d'un métal divalent, par rapport au poids de la matière en polyamide.

11. Solution suivant la revendication 9, qui comprend en outre une composition fluorochimique repoussant l'huile et l'eau.
